

Patented Oct. 5, 1954

2,691,000

# UNITED STATES PATENT OFFICE

2,691,000

## LUBRICATING OILS

John Scotchford Elliott, London, England, assignor to C. C. Wakefield & Company Limited, London, England, a British company

No Drawing, Application April 15, 1952,  
Serial No. 282,472

Claims priority, application Great Britain  
April 23, 1951

13 Claims. (Cl. 252—48.6)

### 1

This invention is for improvements in or relating to lubricants which are to be used under conditions which tend to disrupt the lubricant film, which disruption more particularly takes place when the pressure between the bearing surfaces is very great.

Where the lubricant is required to lubricate surfaces under the above conditions, the film rupture strength becomes more important than the coefficient of friction. For example, under the extreme pressures obtaining in hypoid gears, if the oil film is ruptured, the metal surfaces will contact one with the other, thereby leading to loss of efficiency, excessive wear and ultimately to failure of the mechanism.

There have already been provided lubricants which have a high film-rupture strength. Such lubricants are generally known in the trade as "extreme-pressure" lubricants.

These extreme-pressure lubricants originally consisted of lubricating oil which contained sulphur, either in the form of flowers of sulphur or as a colloidal dispersion. The sulphur, however, was liable to precipitation and it was later proposed to prepare these extreme-pressure lubricants by treating a fatty oil, for example, an animal oil, with thionyl-chloride or with similar reagents, such as sulphur monochloride, sulphur dichloride, etc., and then to add the product of this reaction to a mineral oil.

A theory as to the action of extreme pressure lubricants has been that the sulphur reacts with metallic surfaces and forms a very thin coating of iron sulphide and that this sulphide film is sufficient to prevent the metallic surfaces coming into contact with one another should the lubricant film be ruptured. If this theory is, in fact, correct, then it is obvious that the sulphur contained in the oil must be in such form as to be capable of reacting with the metallic surfaces which it is desired to lubricate. On the other hand, the sulphur compound must not be so reactive as to induce corrosion of the surfaces.

A large number of organic compounds have been proposed for use as extreme pressure agents, including various types of organic di- and polysulphides, and the corresponding derivatives of selenium and tellurium. While the higher polysulphides are very effective in increasing the film rupture strength of the oil in which they are dissolved, they tend to be inherently unstable, corrosive, especially to copper and cuprous materials, and to exert a pro-oxidant effect upon the oil.

The disulphides, on the other hand, usually possess rather poor extreme pressure properties, insufficient to warrant their use except in conjunction with other extreme pressure additives such as organic halogen compounds. Thus, for example, it has been proposed to employ a mix-

### 2

ture of dibenzyl disulphide or of a dialkyl disulphide with a variety of organic chlorine compounds.

It is an object of the present invention to provide lubricating compositions having extreme pressure properties containing additives which do not substantially tend to increase the rate of oxidation of the oils in service.

It is a further specific object of the invention to provide additives capable of substantially increasing the film rupture strength of lubricating oils for turbines and/or hypoid gears without at same time increasing their tendency to oxidise or emulsify with water.

15 Thus at the present time many oils used for turbine lubrication consist of specially selected mineral oil blends stabilised against oxidation by the incorporation of antioxidant additives and containing also additives designed to protect ferrous metal parts against rusting or corrosion by, e. g., sea water. It is of course important that additional additives, incorporated in such oils for the purpose of enhancing their extreme pressure properties, should not interfere in any way 20 with the normal functions of the two foregoing classes of additive. Many turbine oils, especially marine turbine oils used by the Admiralty, are controlled as regards oxidation stability, salt water corrosion of ferrous metals, demulsification 25 value and corrosive action on cuprous metals, by a very rigid specification. It is necessary, therefore, that extreme pressure additives incorporated therein should not adversely affect compliance with its clauses.

30 Many of the more commonly employed extreme pressure additives are detrimental in one or more respects. Thus chlorine compounds generally tend to promote oxidation and are also prone to hydrolysis with the subsequent liberation of hydrochloric acid which accelerates 35 rusting of ferrous metal parts.

Many sulphur compounds are also pro-oxidant, and those which are without effect in this respect usually possess inadequate extreme pressure properties.

40 We have found a class of organic sulphur compounds which possess surprisingly effective extreme pressure properties and which at the same time do not increase oxidation, ferrous metal corrosion or emulsification, and which therefore may be used in turbine oils with impunity.

45 These compounds are the esters of acetic acid substituted in the alpha position by di- or poly-sulphide groups, and the corresponding derivatives of selenium or tellurium and may be represented by the general formula:



50 55 60 where the radical R is an alkyl, aryl or cycloalkyl

radical, X is sulphur, selenium or tellurium and n is 2, 3 or 4.

The radicals R may contain halogen substituents, although as already indicated the presence of halogen is to be avoided if the compounds are to be used in certain applications, particularly in the turbine oils.

It would appear that the presence of ester groups situated in the alpha position to the di- or polysulphide groups exerts an activating influence with the consequent production of extreme pressure properties substantially in excess of those obtainable by the use of the simple aliphatic, aromatic or aryl substituted aliphatic di- or polysulphides.

According to the present invention a lubricating composition comprises a mineral lubricating oil base and a minor proportion, sufficient substantially to increase the load-carrying capacity of the oil, of an ester of acetic acid substituted in the alpha position by sulphur, selenium or tellurium said ester having the general formula



where R is an alkyl, aryl or cycloalkyl radical which may contain halogen substituents, X is sulphur, selenium or tellurium and n is 2, 3 or 4.

The invention includes a turbine oil comprising a mineral lubricating oil base containing agents controlling oxidation stability and corrosion of ferrous metals and including also a minor proportion, sufficient substantially to increase the load-carrying capacity of the oil, of an ester of acetic acid substituted in the alpha position by sulphur, selenium or tellurium said ester having the general formula



where R is an alkyl, aryl or cycloalkyl radical, X is sulphur, selenium or tellurium and n is 2, 3 or 4.

Specific examples of compounds which may be employed as additives in accordance with the present invention are

#### Diethyl dithiodiacetate



#### Di-n-butyl trithiodiacetate



#### Diphenyl dithiodiacetate



#### Di-n-butyl diselenodiacetate



#### Di-n-butyl tetrathiodiacetate



It has been found, surprisingly, that the presence of substituents such as alkyl groups or ester-substituted alkyl groups attached to the

carbon atom adjacent to the radical X results in a considerable loss of load-carrying ability. Thus the presence of unsubstituted —CH<sub>2</sub>— groups appears to be essential, in addition to the presence of ester groups in the alpha position in order to provide the outstanding extreme pressure properties to which reference has been made.

While it is believed that some, at least, of the additive compounds referred to above are new and have not been prepared heretofore, they may be prepared by methods known to the art. Thus, they may be prepared by the reaction of the corresponding  $\alpha$ -chloro or  $\alpha$ -bromo esters with sodium di- or poly-sulphides in alcoholic solution, or by oxidation of the  $\alpha$ -mercapto esters to give the corresponding disulphides, or by reaction of the  $\alpha$ -mercapto esters with sulphur dichloride or sulphur mono-chloride in a non-ionising solvent to give the tri- and tetra-sulphides respectively.

Specific examples of additives employed in the present invention and methods of preparing them are as follows:

#### EXAMPLE I

##### Preparation of di(n-butyl) dithiodiacetate

An alcoholic solution of sodium disulphide was prepared by dissolving 26.4 grams of sodium sulphide crystals Na<sub>2</sub>S.9H<sub>2</sub>O and 3.52 grams of sulphur (0.11 mol in each case) in 150 mls. of 95% alcohol at the boiling point.

The deep red solution so obtained was cooled to about 30 C. and 28 grams (0.1 mol.) of n-butyl monochloroacetate was added dropwise with continuous stirring and cooling maintaining the temperature below about 60° C.

An almost instantaneous exothermic reaction took place and sodium chloride was precipitated.

At the conclusion of the reaction the mixture was diluted with water to about 500 ccs. total volume and the reaction product extracted with petroleum ether.

After washing the extract with water, it was dried over anhydrous sodium sulphate, filtered, and the solvent removed by distillation.

The product was a pale yellow liquid with a characteristic odour.

#### EXAMPLE II

##### Preparation of di(n-butyl) trithiodiacetate

This was prepared precisely as outlined in Example I, except that twice the amount of sulphur was used.

The product resembled the disulphide in appearance.

By adopting the procedure described in Examples I and II, it has been found possible to prepare substantially neutral chlorine-free products without difficulty.

#### EXAMPLE III

##### Preparation of di(n-butyl) tetrathiodiacetate

37.05 grams of n-butyl thioglycolate (0.25 mol.) was dissolved in 100 mls. benzene and cooled below 0° C. in a bath of 50% ice and 50% concentrated hydrochloric acid. 16.88 grams (1/8 mol.) of sulphur monochloride was dissolved in 50 mls. benzene and cooled in the same way.

The n-butyl thioglycolate solution was now added dropwise with stirring, keeping the temperature below 0° C. A brisk reaction took place with evolution of hydrogen chloride. After standing for two hours, the mixture was allowed to warm up to room temperature, the evolution of hydrogen chloride continuing for some hours. The solvent was removed at a temperature not exceeding 25° C.

The product was a yellow liquid.

By methods analogous to those described in Examples I and II, it has been found possible to prepare a variety of compounds falling within the scope of the present invention, some examples of which are as follows:

Diethyl dithiodiacetate, prepared by the method of Example I from ethyl monochloracetate.

(A mixture of the di- and trisulphides in approximately 3:1 ratio containing 29.0% sulphur was actually made.)

Di (2-ethyl hexyl) trithiodiacetate, prepared similarly from 2-ethyl hexyl monochloracetate (as in Example II).

Dicyclohexyl dithiodiacetate, prepared similarly from cyclohexyl monochloracetate.

Di ( $\beta$ -chloroethyl) dithiodiacetate



prepared similarly from  $\beta$ -chloroethyl chloracetate, which was prepared by reacting chloracetyl chloride with ethylene chlorhydrin.

Analysis showed that this product was a mixture of compounds formed by the replacement of some of the terminal chlorine atoms by disulphide groups.

Aryl esters such as diphenyl dithiodiacetate cannot readily be prepared by the foregoing methods as hydrolysis of the esters appears to take place. They may, however, be prepared via the Bunte salts by a method similar to that described by Stoner and Dougherty in the Journal of the American Chemical Society, vol. 63, p. 987 (1941). Thus, for example, phenyl monochloracetate may be reacted in boiling 50% aqueous alcohol with sodium thiosulphate, and the product converted to the disulphide by the addition of iodine.

Yields are usually rather poor and it is therefore generally preferred to employ the alkyl or cycloalkyl esters.

Selenium compounds such as di(n-butyl) diseleno-diacetate may be prepared by reacting the  $\alpha$ -halo ester e. g. n-butyl monochloracetate with sodium or potassium selenosulphate in aqueous alcoholic solution by the method employed by Stoner and Williams in the Journal of the American Chemical Society, vol. 70, page 1113 (1948).

The additives used will of necessity be soluble in the mineral oil base in the proportions in which they are to be employed. The preferred compounds are those which are miscible with oil in all proportions, although others of lower solubility may be satisfactorily used. The oil solubility will necessarily depend upon the nature of the groups R but in general complete miscibility with oil may be achieved by employing as radical R an aliphatic or cycloaliphatic radical having not less than four carbon atoms.

The amounts of the additives employed will depend upon the purpose for which the oil is to be used. Any quantity from the minimum sufficient to impart a substantial increase in film rupture strength up to about 10 per cent may be employed, but in general from about 0.5 per cent to about 2.0 per cent is contemplated, especially for use in turbine oils.

The so-called inhibited turbine oils to which the compounds of this invention may be added normally contain antioxidant additives which may be of the alkylated phenol type, e. g., tertiary butyl cresol, 2:4 dimethyl-6-tertiary butyl phenol, 2:6 di-tertiary butyl-p-cresol, or secondary aromatic amines, e. g., diphenylamine,

phenyl- $\alpha$ -naphthylamine, phenyl- $\beta$ -naphthylamine, and also anti-rusting additives which may be of various types, one preferred class of additives being the acid esters of the long-chain mono esters of polyhydric alcohols described in patent application No. 191,166.

Some of the additives contemplated, notably the tri- and higher polysulphides, tend to be somewhat corrosive to copper and cuprous alloys at elevated temperatures. In such cases, it is desirable to incorporate also a copper stain inhibitor of the type disclosed in Patent No. 2,414,257, e. g., mercaptobenzothiazole, benzothiazole disulphide, benzothiazole hydroxymethyl sulphide, or tetramethyl or tetraethyl thiram disulphide.

The additives of the present invention may, if desired, be employed in conjunction with organic halogenated compounds in mineral lubricating oils to provide, for example, extreme pressure lubricants for hypoid gears. Oils containing such combinations of additives are capable of withstanding higher loads than oils which contain only the sulphur compound. As already stated, however, the presence of halogen compounds in turbine oils is undesirable.

To demonstrate the effectiveness of the compounds of the present invention as extreme pressure agents, tests were carried out on the well-known Society of Automotive Engineers (S. A. E.) Testing Machine, a description of which may be found in the Co-ordinating Research Council (C. R. C.) Handbook (1946) on pages 458-462. This machine was operated at 500 R. P. M. using a standard loading rate of 75 to 85 lbs./sec. and rubbing ratio of 14.6:1.

The additives were dissolved in a mineral oil blend (oil A) consisting of 70% of a mineral oil having a viscosity of about 170 seconds Redwood at 140° F. and 30% of a solvent refined mineral oil having a viscosity of about 65 seconds Redwood at 140° F.

The results obtained are tabulated below, the failure loads recorded being in general the mean of several tests.

Certain other closely related compounds were tested at the same time in order to demonstrate the superiority of the compounds of the present invention. In the majority of instances the percentages of additive used were adjusted to provide an amount of added sulphur of between 0.23 and 0.28 per cent.

| 55 | Compound                                                     | Percent | Percent sulphur provided by the additive | Failure load (lbs.)                        |
|----|--------------------------------------------------------------|---------|------------------------------------------|--------------------------------------------|
| 60 | 1. None.                                                     |         |                                          | Approx. 70.<br>230.                        |
|    | 2. Di-(n-butyl) dithiodiacetate.                             | 1.0     | 0.23                                     |                                            |
|    | 3. Di(n-butyl)trithiodiacetate.                              | 1.0     | 0.18                                     | 280.                                       |
|    | 4. Di(n-butyl)tetrahiodiacetate.                             | 0.75    | 0.27                                     | 275.                                       |
|    | 5. Di( $\beta$ -chloroethyl)dithiodiacetate. <sup>1</sup>    | 1.0     | 0.36                                     | 310.                                       |
|    | 6. Di(n-butyl)diselenodiacetate.                             | 1.0     | 0.34                                     | 345.                                       |
|    | 7. Dibenzyl disulphide.                                      | 1.0     | 0.26                                     | 300.                                       |
|    | 8. Dibenzyl trisulphide (31.7% S).                           | 0.8     | 0.25                                     | 115.<br>125.                               |
|    | 9. Diphenyl disulphide.                                      | 1.0     | 0.26                                     | 90.                                        |
|    | 10. Di(n-butyl) monothiodiacetate.                           | 2.5     | 0.25                                     | 100.                                       |
| 70 | 11. Di(n-butyl) di $\beta$ -thiodi-<br>proponate.            | 1.5     | 0.32                                     | scattered results<br>not exceeding<br>120. |
|    | 12. Di(n-butyl)dithiobis<br>( $\alpha$ -dimethyl) diacetate. | 1.5     | 0.24                                     | 90.                                        |

<sup>1</sup> This compound had a rather limited oil-solubility.

It will be apparent from the foregoing tests that the compounds of the present invention (numbers 2 to 6) possess a marked advantage over:

(a) Conventional di- and polysulphides (numbers 7 to 9);

(b) The corresponding monosulphides (number 10);

(c) A closely related ester containing a disulphide group in the  $\beta$ -position to the ester group instead of the  $\alpha$ -position (number 11), and

(d) A compound containing alkyl substituents attached to the disulphide group (number 12).

In order to obtain the best results, it would appear desirable to have the radicals R consisting of relatively short alkyl chains, the introduction of large or cyclic groups tending to reduce load-carrying capacity. Thus it is preferred that the radicals R shall consist of alkyl radicals having not more than six carbon atoms.

To illustrate the effectiveness of the compounds of the present invention when employed for the purpose of imparting extreme pressure properties to turbine oils, an inhibited turbine oil conforming to British Admiralty Specification OM.88 was selected (oil B). This consisted of an oil similar to oil A. containing 0.5% of a secondary aromatic amine type oxidation inhibitor and 0.07% of a ferrous metal corrosion inhibitor consisting of ethylene glycol mono-naphthenate acid phthalate.

The following table illustrates the effect of additives of the present invention on the properties of oil B:

| Additives                                                                               | Acidity,<br>milligrams<br>KOH/gm. | Demulsi-<br>fication<br>value | Oxidation Test                  |                                                  | Salt Water<br>Corrosion<br>test | S. A. E.<br>Machine<br>Test (500<br>R. P. M.) |
|-----------------------------------------------------------------------------------------|-----------------------------------|-------------------------------|---------------------------------|--------------------------------------------------|---------------------------------|-----------------------------------------------|
|                                                                                         |                                   |                               | Acidity<br>after ox-<br>idation | Demulsi-<br>fication<br>Value after<br>oxidation |                                 |                                               |
| 1. None.....                                                                            | 0.08                              | Seconds                       |                                 | Seconds                                          | No rusting.....                 | 150                                           |
| 2. Diethyl-dithio-diacetate (2%).....                                                   | 0.17                              | 180                           | 0.17                            | 540                                              | No rusting.....                 | 340                                           |
| 3. Di( <i>n</i> -butyl)trithio-diacetate (1.5%) + benzothiazole disulphide (0.1%).....  | 0.08                              | 180                           | 0.14                            | 330                                              | No rusting.....                 | 250                                           |
| 4. Di( <i>n</i> -butyl)trithio-diacetate (1.0%) + mercaptobenzothiazole (0.05%).....    | 0.20                              | 180                           | 0.17                            | 480                                              | .....do.....                    | 275                                           |
| 5. Dicyclohexyl dithio-diacetate (1.5%).....                                            | 0.08                              | 135                           |                                 |                                                  |                                 |                                               |
| 6. Di( <i>n</i> -butyl)diseleno-diacetate (1.0%) + benzothiazole disulphide (0.1%)..... | 0.15                              | 150                           | 0.08                            | 225                                              | Very slight<br>rusting.....     |                                               |

<sup>1</sup> The somewhat high acidity in this instance was due to the presence of a trace of acid in the additive.

The methods employed for determining the various values quoted above were standard methods described in the "Standard Methods for Testing Petroleum and its Products," and having the following references:

Acidity, I. P. 1/46, Method A (page 1—1951 edition).

Demulsification value, I. P. 19/51 (page 117—1951 edition).

Oxidation test, I. P. 114/47 (page 363—1951 edition).

Salt water corrosion test, I. P. 125/51 (1951 edition, page 390) (modified in respect of salt water composition and duration, to comply with the requirements of British Admiralty Specification OM.88).

It will be seen from the foregoing tests that the additives of the present invention not only greatly enhanced the load-carrying capacity of the turbine oil in which they were dissolved, but also left unaffected the essential properties of the oil, i. e., low acidity, low demulsification value, high resistance to oxidation and ability to inhibit corrosion of ferrous metals by salt water.

In order to eliminate completely all tendency

of the oils to stain copper under the conditions of the standard copper strip corrosion test (I. P. 64/51, Procedure C, page 550, 1951 edition), i. e., immersion for 3 hours at 100° C., it has been found necessary in general to employ a copper stain inhibitor of the type already described, examples of satisfactory combinations of additives having been quoted in the foregoing table. In this connection it is generally preferred to use the di- and tri-sulphides since the activity of the sulphur in the tetra-sulphides is greater and more difficult to control.

Comparative tests on certain of the oils were obtained by the use of a high speed disc testing machine in which two discs of En. 36 case-hardened steel of diameter 8" and 4", respectively, were rotated in contact with one another at speeds of 1800 and 7200 revolutions per minute, respectively, the sliding velocity being 3775 feet per minute. The discs were immersed in the oil under test, which was maintained at 155–165° F., and the load on the discs was gradually increased until scuffing took place. The results were recorded as Sc loads at the incidence of scuffing, the definition of the term Sc being:

Pounds load per inch of length of line of contact  
(Relative radius of curvature)<sup>0.8</sup>

Six tests were carried out on each of the oils tabulated below, and the mean Sc loads quoted for each oil. Oil C was a typical turbine oil of similar viscosity to oil B and containing anti-oxidant and rust inhibitors.

| Oil                                                                                              | Mean Sc<br>load at<br>scuffing<br>(lbs.) |
|--------------------------------------------------------------------------------------------------|------------------------------------------|
| 1. Oil C.....                                                                                    | 1,300.                                   |
| 2. Oil B +<br>[1.0% Di( <i>n</i> -butyl) trithiodiacetate<br>0.05% Mercaptobenzothiazole.....]   | over 12,550.                             |
| 3. Oil B +<br>[1.5% Di( <i>n</i> -butyl) trithiodiacetate<br>0.1% Benzothiazole disulphide.....] | over 12,550.                             |

In the case of oils 2 and 3, no scuffing was experienced in three and six tests, respectively, up to a limit of 12,550 lbs., after which the tests were discontinued. The other three tests on oil 2 were terminated at lower Sc loads, without any scuffing having occurred.

To provide illustrations of lubricating oil compositions suitable for use as extreme pressure lubricants for hypoid gears, compounds of the present invention were dissolved in a relatively viscous mineral oil blend designated oil D, which consisted of 27 parts by weight of a conventionally refined Pennsylvanian bright stock of viscosity 600 seconds Redwood at 140° F., 34 parts of a conventionally refined Mid-Continent

bright stock of viscosity 750 seconds Redwood at 140° F., 3 parts of a solvent refined neutral oil of viscosity 65 seconds Redwood at 140° F., and 23 parts of a solvent refined paraffinic distillate of similar viscosity. Typical blends were subjected to test on the S. A. E. machine already described, but operated at 750 R. P. M. instead of 500 R. P. M. as previously:

|        | Oil                                        | Failure load (lbs.) |
|--------|--------------------------------------------|---------------------|
| A..... | 89.8% Oil D.....                           | 435.                |
|        | 8% chlorinated paraffin wax.....           |                     |
|        | (40% chlorine).....                        |                     |
|        | 2% Di(n-butyl) dithiodiacetate.....        |                     |
| B..... | 0.2% Mercaptobenzothiazole.....            |                     |
|        | 01.9% Oil D.....                           |                     |
|        | 5% Hexachlorethane.....                    |                     |
|        | 3% Di(2-ethyl hexyl) trithiodiacetate..... |                     |
|        | 0.1% Tetraethyl thiuram disulphide.....    | 405.                |

The normal requirement for a good extreme pressure lubricant for hypoid gears is that it should withstand loads up to 350 lbs. under these conditions.

I claim:

1. A lubricating composition comprising a mineral oil containing a small amount sufficient to increase the load-carrying capacity of the oil of an ester of acetic acid substituted in the alpha position by an element selected from the group consisting of sulphur and selenium, said ester having the general formula



in which R is a radical selected from the group consisting of alkyl, aryl and cycloalkyl radicals, X is an element selected from the group consisting of sulphur and selenium and n is an integer from 2 to 4 inclusive.

2. A lubricating composition comprising a mineral oil containing a small amount sufficient to increase the load-carrying capacity of the oil of an ester of acetic acid substituted in the alpha position by an element selected from the group consisting of sulphur and selenium, said ester having the general formula



in which R is a chlorine containing radical selected from the group consisting of alkyl, aryl and cycloalkyl radicals, X is an element selected from the group consisting of sulphur and selenium and n is an integer from 2 to 4 inclusive.

3. A lubricating composition comprising a mineral oil containing about 0.5% to about 10% by weight of an ester of acetic acid substituted in the alpha position by an element selected from the group consisting of sulphur and selenium, said ester having the general formula



in which R is a radical selected from the group consisting of alkyl, aryl and cycloalkyl radicals, X is an element selected from the group consisting of sulphur and selenium and n is an integer from 2 to 4 inclusive.

4. A lubricating composition comprising a mineral oil containing from 0.5% to 2.0% by weight of an ester of acetic acid substituted in the alpha position by an element selected from the group consisting of sulphur and selenium, said ester having the general formula



in which R is a radical selected from the group consisting of alkyl, aryl and cycloalkyl radicals, X is an element selected from the group consisting of sulphur and selenium and n is an integer from 5 to 4 inclusive.

5. A lubricating composition comprising a mineral oil containing a small amount sufficient to increase the load-carrying capacity of the oil of an ester of acetic acid substituted in the alpha position by an element selected from the group consisting of sulphur and selenium, said ester having the general formula



15 in which R is an alkyl radical containing not more than six carbon atoms X is an element selected from the group consisting of sulphur and selenium and n is an integer from 2 to 4 inclusive.

6. A lubricating composition comprising a mineral oil containing from 0.5% to 2.0% by weight of an ester of acetic acid substituted in the alpha position by an element selected from the group consisting of sulphur and selenium, said ester having the general formula



in which R is an alkyl radical containing not more than six carbon atoms X is an element selected from the group consists of sulphur and selenium and n is an integer from 2 to 4 inclusive.

7. A lubricating composition as claimed in claim 1 in which there is also incorporated a small amount of a compound selected from the group consisting of mercapto-arylene-thiazoles and derivatives of mercapto-arylene-thiazoles.

8. A lubricating composition as claimed in claim 1 in which there is also incorporated a small amount of an alkyl thiuram disulphide.

9. A lubricating composition as claimed in claim 1 in which there is also incorporated a small amount of benzothiazole disulphide.

10. A lubricating composition comprising a mineral oil containing as an additive from 0.5% to 2.0% by weight of di(n-butyl) dithiodiacetate.

11. A lubricating composition comprising a mineral oil containing as an additive from 0.5% to 2.0% by weight of di(n-butyl) trithiodiacetate.

12. A turbine oil comprising a mineral oil containing agents controlling oxidation stability and corrosion of ferrous metals and including also a small amount sufficient to increase the load-carrying capacity of the oil of an ester of acetic acid substituted in the alpha position by an element selected from the group consisting of sulphur and selenium, said ester having the general formula



in which R is a radical selected from the group consisting of alkyl, aryl and cycloalkyl radicals, X is an element selected from the group consisting of sulphur and selenium and n is an integer from 2 to 4 inclusive.

13. An extreme pressure lubricant comprising a lubricating oil composition as claimed in claim 1 and including in addition to the ester of acetic acid an organic halogenated compound.

#### References Cited in the file of this patent

#### UNITED STATES PATENTS

| Number    | Name           | Date          |
|-----------|----------------|---------------|
| 2,073,841 | Humphreys      | Mar. 16, 1937 |
| 2,317,666 | Burwell        | Apr. 27, 1943 |
| 2,467,303 | Frank          | Apr. 12, 1949 |
| 2,503,401 | Mattano et al. | Apr. 11, 1950 |
| 2,649,416 | Richter et al. | Aug. 18, 1953 |